

June 12, 1928.

H. F. ALBRIGHT

1,672,973

## METHOD FOR COATING CORES

Filed Feb. 3, 1923



*Inventor  
Henry F. Albright  
by H. Patterson. Atty.*

## UNITED STATES PATENT OFFICE.

HENRY FLEETWOOD ALBRIGHT, OF OAK PARK, ILLINOIS, ASSIGNOR TO WESTERN ELECTRIC COMPANY, INCORPORATED, OF NEW YORK, N. Y., A CORPORATION OF NEW YORK.

## METHOD FOR COATING CORES.

Application filed February 3, 1923. Serial No. 616,662.

This invention relates to a method and apparatus for coating cores.

The object of the invention is to produce a core having a continuous, uniform, and 5 homogeneous coating of fibrous material.

Briefly, the method consists in moistening a strip or strips of paper or other suitable fibrous material, pressing the wet strip or strips upon the core to be coated, forming 10 the deposited material while still moist around the core so that it constitutes a smooth, continuous and homogeneous coating therefor, and then removing substantially all of the moisture from said coating.

15 The present method may be employed to advantage for insulating electrical conductors but it is to be understood that it is not limited to this purpose, but only in so far as is defined by the appended claims. Where 20 the method is used for insulating electrical conductors, paper or other fibrous material made from manila, wood, rag, cotton, esparto, jute, hemp, and asbestos may be employed as the coating material, but other 25 materials than those specified may be used without departing from the spirit and scope of the invention.

The drawings illustrate an apparatus by 30 which the method may be practiced, the apparatus being especially designed for coating a core in strand form, but it is to be understood that other apparatus may be devised for coating cores in other forms without departing from the spirit and scope of 35 the invention.

In the accompanying drawings:

Fig. 1 is a side elevation of a preferred 40 apparatus for performing the process;

Fig. 2 is an enlarged fragmentary top plan view of the apparatus shown in Fig. 1, and

45 Figs. 3, 4 and 5 are enlarged vertical sectional views showing the construction of the coating upon its delivery from the squeezing rolls, during the forming operation, and after the forming operation is completed respectively.

The steps of the method will be readily 50 understood from a detailed description of the apparatus by which the method may be practiced.

Referring to the drawings in detail in 55 which like reference numerals designate similar parts, the core to be coated is fed

from a supply 20 over an idler roll 21 and 55 thence between a pair of squeeze rolls 22, the supply spool 20 and rolls 21 and 22 being suitably supported upon a framework 23 which supports all of the elements of the apparatus. Two reels 24 and 25, each containing a supply of paper or other suitable fibrous material in strip form, are supported by the framework 23 and disposed between the rolls 21 and 22. The reel 24 is mounted above the core to be coated and the reel 25 supported below the said core, so that when the paper strips are drawn from these rolls between the squeeze rolls 22, the strips will be positioned upon diametrically opposite sides of the core. The rolls 22 serve to 60 65 squeeze the two strips of paper and core into close contact.

From the squeeze rolls 22 the core and 70 paper strips are passed around rolls 26 and 27 submerged in a moistening fluid within 75 a tank 28 or other suitable receptacle carried by the framework 23. The moistening fluid contained within the tank 28 is preferably water, but other fluids may be employed, either of an adhesive or non-adhesive 80 nature, and either waterproofing or non-waterproofing in character, without departing from the spirit and scope of the invention. The strips of paper in passing through the water are moistened sufficiently 85 to soften the fibers of the paper so that when the strips are passed between squeeze rolls 29 the fibers in each of the paper strips are felted together to some extent so that they 90 form an envelope enclosing the conductor, as shown in Fig. 3. The squeeze rolls 29 also serve to remove the surplus moisture from the moistened paper strips.

From the squeeze rolls 29 the core with 95 its envelope covering is passed through a forming mechanism 30. The mechanism shown is identical with the forming mechanism fully illustrated and described in a co-pending application of Walker and March, Serial No. 547,923, filed March 29, 100 1922, and for a detailed disclosure of the construction of this mechanism reference is made to the application above noted. The forming mechanism wraps the projecting edges of the ribbons around the core and 105 around each other, the appearance of the coating after it is first acted on by the forming mechanism and after the forming action

is completed being clearly shown in Figs. 4 and 5. The former causes an intermingling of the softened or somewhat adhesive fibers so that a substantially homogeneous coating is produced which conforms to the shape of the core.

The core with the formed coating is drawn from the forming mechanism and subjected to a mechanism for thoroughly drying out the coating. This means shown for performing this step in the process are a pair of wide hollow drums 31 and 32 internally heated and having a plurality of grooves 33 formed thereon (Fig. 2) which receive the coated core, guides (not shown) being provided for directing the core over first one drum and then the other until it has traversed all of the grooves of both drums, after which it is stored on a storage reel 34.

20 The storage reel 34, drums 31 and 32, forming mechanism 30, and squeeze rolls 29 are all connected with a suitable source of power for actuating them to feed the core to be coated from the supply reel 20 through 25 the various mechanisms above described and onto the storage reel 34.

In the mechanism shown in the drawings means is provided for coating a single core, but it is to be understood that by duplicating the various elements of the mechanism a plurality of cores may be accommodated. Where it is desired to coat a plurality of cores simultaneously the reels 24 and 25 may be designed to accommodate

wide strips of paper which may be subsequently slit into ribbons associated with each core. Any suitable slitting mechanism may be employed located at any suitable point, as for instance prior to or subsequent to the passage of the paper through the moistening tank 28.

What is claimed is:

1. A method of coating a core in strand form, which consists in applying a strip of paper to a core to be coated, applying water to the strip of paper, and wrapping the strip around the core and intermingling, felting and matting the fibers of said paper so that it constitutes a continuous and homogeneous coating therefor which is retained thereon solely by the intermingling, felting and matting of the fibers.

2. A method of coating a core in strand form, which consists in applying a strip of paper to a core to be coated, applying water to the strip of paper, wrapping the strip around the core and intermingling, felting and matting the fibers of said paper so that it constitutes a continuous and homogeneous coating therefor which is retained thereon solely by the intermingling, felting and matting of the fibers, and then drying the core and its paper coating.

In witness whereof, I hereunto subscribe my name this 24th day of January, A. D., 1923.

HENRY FLEETWOOD ALBRIGHT.